

# UNITED STATES PATENT OFFICE.

WILLIAM C. BLATZ, OF WILMINGTON, DELAWARE, ASSIGNOR OF ONE-HALF TO JOHN B. BLATZ, OF PHILADELPHIA, PENNSYLVANIA.

## MANUFACTURE OF LEATHER.

1,334,216.

Specification of Letters Patent. Patented Mar. 16, 1920.

No Drawing. Application filed February 5, 1917. Serial No. 146,734. Renewed April 24, 1919. Serial No. 292,420.

*To all whom it may concern:*

Be it known that I, WILLIAM C. BLATZ, a citizen of the United States, and a resident of Wilmington, New Castle county, Delaware, have invented certain Improvements 5 in the Manufacture of Leather, of which the following is a specification.

My invention relates to the manufacture 10 of leather, and the object of my present invention is to produce a white leather available for general use in the arts and particularly valuable for the manufacture of shoes and other forms of footwear.

My invention comprises the precipitation 15 of an insoluble barium salt within and upon the surface, body and fibers of a skin or hide, during or subsequent to the tanning or tawing operation, for the purpose of producing a white leather; the barium salt not only precipitating in a white state, thus determining and fixing the final color of the leather produced from the hide or skin operated upon, but also neutralizing any coloration 20 that may have been imparted by the tanning or tawing operation, whether the latter includes a chrome treatment or not, so that the leather, when finished, is a pure white product.

The purpose of my invention is the precipitation 30 of an insoluble barium salt, within and upon the surface, body and fibers of skins and hides tawed or tanned by any process involving a chrome treatment or a modified chrome treatment, and while I propose to carry this into effect in connection 35 with hides and skins tawed or tanned by a combination process which may include an alum treatment followed by a chrome treatment, I do not wish to be limited to any particular method or process of tanning or 40 tawing a skin or hide involving the use of chrome preliminary to carrying out my improved process of precipitating an insoluble barium salt within and upon the surface, body and fibers of the skins or hides for the 45 purpose of producing a white leather product.

The improved white product made in accordance with my invention, differing from 50 many, if not all, white leathers, including alum-tawed leathers, is susceptible of receiving a gloss or polish under a glazing operation, and this glazing operation has the ef-

fect of not only improving the character of the leather, but also of closing the pores of 55 the skin or hide and increasing the moisture-resistant properties of the final leather product.

My invention is based upon the discovery 60 that an insoluble barium salt may be precipitated within and upon the surface, body and fibers of the skin or hide by subjecting the same at a certain stage of the tanning or tawing treatment, or after the tanning or tawing treatment is completed, to the action 65 of a soluble salt of barium with a salt (such as sodium sulfate or its equivalent for the desired purpose) capable of reacting therewith to produce an insoluble precipitate of barium in a white state; the resulting reaction precipitating the barium salt within 70 and upon the surface, body and fibers of the skin or hide undergoing treatment and retaining it in the final leather product resulting from the complete treatment of such 75 hide or skin. Any other salts that may be formed have no effect upon the skin or hide under treatment, and usually pass to waste.

The precipitation of an insoluble barium salt within and upon the surface, body and 80 fibers of the skin or hide during or following the process of transforming the same into leather, produces a condition of whiteness that is permanent, since the barium salt is insoluble and can not be washed from the 85 finished leather.

While it is possible that other salts including metallic salts, or the salts of other alkaline earth metals may be precipitated 90 within and upon the surface, body and fibers of leather for the purpose of producing a white product, barium possesses a number of characteristics which make it peculiarly valuable and desirable for the described purpose. In the first place, it is one of the most 95 inert salts known, being insoluble in water and substantially insoluble in acids, and it precipitates absolutely white in the skin or hide to which it is subjected under my improved method or process of treatment. 100

In carrying out my improved process for the production of white leather from skins and hides, I may proceed substantially as follows:

The skins, after being prepared for tan- 105 ning or tawing by any method, which prep-

aration may include the usual puring in any suitable bate; slating to remove the fine hairs, and washing in water, may be subjected to the action of a tawing paste of well known character including oil; egg yolk; flour; alum, and common salt, preferably in a drum, and the treatment of the skins following the application of the tawing paste may be substantially that of any of the chrome tawing or tanning processes now in common use.

Prior to the usual finishing steps to which the hides or skins are subjected when the tanning or tawing treatment proceeds in the usual manner, and the tanning or tawing operation being complete or substantially so, the treatment which characterizes my invention may be commenced, and to the usual hypo-solution which, for one hundred (100) pounds of skins or hides, may consist approximately of

Hyposulfite of soda 15.0%  
Muriatic (or sulfuric) acid .5%

with sufficient water to provide a bath having a volume of approximately fifteen (15) gallons; (the amount of hypo being somewhat greater than that usually employed,) I add about 6% of a soluble salt such as potassium sulfate; sodium sulfate; magnesium sulfate; ammonium oxalate; etc., etc., or any equivalent salt capable of performing the desired function. This addition is made to the usual hypo-solution employed in the tanning process, or what may be termed a "spent" solution of the same after the usual hypo treatment of the hides or skins. The skins are then drummed in this special solution or bath for approximately three (3) to four (4) hours, and may remain in the same over night.

The special hypo-solution is then drained off, and about 11% of a barium salt in solution in approximately six (6) gallons of water is placed in the drum; and the skins are drummed for a short period of time: the barium salt reacting with any soluble salt left in the bath, after which the excess solution or liquor is drained off. Following this treatment, about 7% of a suitable soluble salt (such as indicated above or any equivalent capable of performing the desired function) capable of reacting with the barium salt to form an insoluble precipitate, in solution in approximately six (6) gallons of water, is placed in the drum, and the skins are drummed in this bath for about one (1) hour, after which about 11% of the barium salt employed in solution in approximately six (6) gallons of water is added to the bath in the drum, and the skins are again drummed for a short period of time.

This alternating treatment of the tanned or tawed skins or hides for proper periods of time with the barium salt and a salt capa-

ble of producing an insoluble barium precipitate, separately and together, both of which agents may be in excess, insures a complete precipitation of an insoluble barium salt within and upon the surface, body and fibers of the skin or hide undergoing treatment, with the resulting whiteness desired, and after the final precipitation the skins are taken out of the drum, struck out in the usual way; dried, and staked. The skins so prepared are permanently white leather, ready for the market or, if desired, they may be subjected to a final glazing or ironing operation. My improved white leather when glazed is a substantially moisture-resistant product.

If desirable for any reason, the skins may be subjected to a fat-liquor treatment to soften them should they be harsh or in a condition that would justify application of the fat-liquor treatment, before being dried out preliminary to the staking operation and the subsequent ironing or glazing operations.

It will be understood, of course, that I may employ a two-bath method of chrome tawing or tanning for the preliminary treatment of the skins, or a one-bath process of any of the well known types, or the usual basic chrome tannage, and while the steps of any usual chrome tannage process may be followed and the materials of such process employed in the tawing or tanning or other treatment of the skins or hides prior to the precipitation of an insoluble barium salt, in such skins or hides, the amount of such materials used is considerably modified; for instance less bichromate of potash, (or soda) and acid (muriatic or sulfuric) may be used, with a considerably greater quantity of hyposulfite of soda than is employed with the usual chrome tannage.

My improved leather product may be described as a "chrome-tanned white leather." I am aware that attempts have been made to produce white leather from chrome-tanned skins but without success, and in all prior efforts to produce white leather, no practical use has been made of chrome tannage on account of the coloring imparted by the chrome.

I have succeeded in producing a permanent white leather from chrome-tanned skins through a new and original process which comprises: (a), reduction of the amount of color resulting from the regular chrome process, and (b), an impregnation of the skin with an insoluble white precipitate, barium being preferred. The white leather obtained by this method will withstand the glazing operation employed in the manufacture of ordinary glazed kid, and is improved by such glazing.

The white leather made in accordance with my invention will not only withstand washing with a cloth wet with water but is,

practically speaking, a white washable leather. For the making of white shoes, whether employed for the complete upper or for the top alone, it is decidedly superior to 5 any of the so-called white leathers heretofore manufactured.

As this application possesses matter in common with an application filed by me November 16, 1916, Serial No. 131,707, it is to 10 be treated as a continuation of said prior application as far as the common subject-matter is concerned.

I claim:

1. The process of treating skins or hides 15 for the production of white leather therefrom, which comprises tanning or tawing the same by a chrome treatment, and then precipitating an insoluble white salt of one of the alkaline earth metals within and 20 upon the surface, body and fibers of the skins or hides to determine and fix the whiteness of the finished product.

2. The process of treating skins or hides 25 for the production of white leather therefrom, which comprises subjecting them to alum-tannage, then to chrome treatment, and then precipitating an insoluble white salt of one of the alkaline earth metals within and upon the surface, body and 30 fibers of the skins or hides to determine and fix the whiteness of the finished product.

3. The process of treating skins or hides 35 for the production of white leather therefrom, which comprises tanning or tawing the same by a modified chrome treatment, and then precipitating an insoluble white salt of one of the alkaline earth metals within and upon the surface, body and fibers of the skins or hides to determine and 40 fix the whiteness of the finished product.

4. The process of treating skins or hides 45 for the production of white leather therefrom, which comprises subjecting them to a modified alum-treatment, then to a modified chrome treatment, and then precipitating an insoluble white salt of one of the alkaline earth metals within and upon the surface, body and fibers of the skins or hides to determine and fix the whiteness of the 50 finished product.

5. The process of producing white leather, 55 which comprises tawing or tanning skins or hides by a chrome treatment, and then precipitating an insoluble barium salt within and upon the surface, body and fibers of the same.

6. The process of treating skins or hides 60 for the production of white leather therefrom, which comprises subjecting them to alum tannage, then to chrome treatment, and finally to the successive action of a barium salt and a salt capable of precipitating the barium salt in an insoluble state within and upon the surface, body and fibers 65 of the skins or hides.

7. The process of treating skins or hides, 70 which comprises subjecting them to a modified chrome treatment whereby the usual chrome coloration is modified, and then to the successive action of a barium salt and a salt capable of precipitating the barium salt in an insoluble state within and upon the surface, body and fibers of the skins or hides to produce a white leather.

8. The process of treating skins or hides 75 for the production of white washable glazed leather therefrom, which comprises subjecting them to chrome treatment, then to the successive action of a barium salt and a salt capable of precipitating the 80 barium in an insoluble state within and upon the surface, body and fibers of the skins or hides, drying and finishing the skins or hides, and then glazing the same.

9. The process of treating skins or hides 85 for the production of white washable glazed leather therefrom, which comprises subjecting them to alum tannage, then to chrome treatment, then to the successive action of a barium salt and a salt capable 90 of precipitating the barium salt in an insoluble state within and upon the surface, body and fibers of the skins or hides, drying and finishing the skins or hides, and then glazing the same. 95

10. The process of treating skins or hides for the production of white washable glazed leather, which comprises subjecting them to a modified chrome treatment whereby the usual chrome coloration is modified, then 100 to the successive action of a barium salt and a salt capable of precipitating the barium in an insoluble state within and upon the surface, body and fibers of the skins or hides, drying and finishing the skins or 105 hides, and finally glazing the same.

11. The process of treating skins or hides 110 for the production of white leather, which comprises tawing or tanning the same by a chrome treatment, and then subjecting the skins or hides to the successive action of a soluble sulfate and barium chloride ( $BaCl_2$ ) whereby barium sulfate is precipitated within and upon the surface, body and fibers of the skins or hides. 115

12. The process of treating skins or hides 120 for the production of white leather, which comprises tawing or tanning the same by a chrome treatment, and then subjecting the skins or hides to the successive action of sodium sulfate ( $Na_2SO_4$ ) and barium chloride ( $BaCl_2$ ) whereby barium sulfate is precipitated within and upon the surface, body and fibers of the skins or hides.

13. The process of treating skins or hides 125 for the production of leather therefrom, which comprises subjecting them to alum-tannage, then to chrome treatment, and finally to the successive action of a soluble sulfate and barium chloride ( $BaCl_2$ ), where- 130

by barium sulfate is precipitated within and upon the surface body and fibers of the skins or hides.

14. The process of treating skins or hides for the production of leather therefrom, which comprises subjecting them to alum-tannage, then to chrome treatment, and finally to the successive action of sodium sulfate ( $Na_2SO_4$ ) and barium chlorid ( $BaCl_2$ ) whereby barium sulfate is precipitated within and upon the surface, body and fibers of the skins or hides.

15. The process of treating skins or hides, which comprises subjecting them to a modified alum-treatment, then to a modified chrome treatment, and finally to the successive action of a soluble sulfate and barium chlorid ( $BaCl_2$ ) whereby barium sulfate is precipitated within and upon the surface, body and fibers of the skins or hides.

16. The process of treating skins or hides, which comprises subjecting them to a modified alum-treatment, then to a modified chrome treatment, and finally to the successive action of sodium sulfate ( $Na_2SO_4$ ) and barium chlorid ( $BaCl_2$ ) whereby barium sulfate is precipitated within and upon the surface, body and fibers of the skins or hides.

17. The method or process of producing white glazed leather, which comprises tawing or tanning skins or hides by a chrome treatment, then subjecting the skins or hides to the successive action of sodium sulfate ( $Na_2SO_4$ ) and barium chlorid ( $BaCl_2$ ) whereby the surface, body and fibers of the skins or hides are impregnated with barium in an insoluble state; such impregnation determining and fixing the whiteness of the finished product, drying and finishing the skins or hides, and finally glazing the same.

18. The method or process of producing white glazed leather, which comprises subjecting skins or hides to alum-tannage, then to chrome treatment, then to the successive action of sodium sulfate ( $Na_2SO_4$ ) and barium chlorid ( $BaCl_2$ ) whereby the surface, body and fibers of the skins or hides are impregnated with barium in an insoluble state; such impregnation determining and fixing the whiteness of the finished product, drying and finishing the skins or hides, and finally glazing the same.

19. In the process of tawing or tanning skins or hides, the step which comprises the

precipitation of an insoluble white salt of one of the alkaline earth metals within and upon the surface, body and fibers of a chrome-treated skin or hide to produce a white leather.

20. In the process of tawing or tanning skins or hides, the step which comprises the precipitation of barium sulfate within and upon the surface, body and fibers of a chrome-treated skin or hide to produce a white leather.

21. As a new article of manufacture, white leather made from chrome-treated skins or hides and having its surface, body and fibers impregnated with an insoluble white salt of one of the alkaline earth metals.

22. As a new article of manufacture, white leather made from chrome-treated skins or hides having its surface, body and fibers impregnated with a barium salt in an insoluble state to determine and fix the whiteness of the same.

23. As a new article of manufacture, white leather made from chrome-treated skins or hides and having its surface, body and fibers impregnated with barium sulfate.

24. As a new article of manufacture, glazed white leather made from chrome-treated skins or hides and having its surface, body and fibers impregnated with a barium salt in an insoluble state.

25. As a new article of manufacture, alum-chrome-tanned leather white in color and having its surface, body and fibers impregnated with a barium salt in an insoluble state to determine and fix the whiteness of the same.

26. As a new article of manufacture, a white chrome-tanned leather, unchangeable in color by washing operations, and having its surface, body and fibers impregnated with a barium salt in an insoluble state.

27. As a new article of manufacture, glazed white washable leather made from chrome-treated skins or hides and having its surface, body and fibers impregnated with a barium salt in an insoluble state.

28. As a new article of manufacture, glazed white washable leather made from alum-chrome-treated skins or hides and having its surface, body and fibers impregnated with a barium salt in an insoluble state.

WILLIAM C. BLATZ.